

Nov. 14, 1933.

F. W. MOSTERTZ

1,934,942

LOOP PILE FABRIC

Filed Jan. 20, 1933

Fig. 1.



Fig. 2.



Fig. 3.



WITNESSES:

Otto L.  
A. M. Ward

INVENTOR

Ferdinand W. Mostertz

BY  
Joshua D. Harris  
HIS ATTORNEY

## UNITED STATES PATENT OFFICE

1,934,942

## LOOP PILE FABRIC

Ferdinand W. Mostertz, Philadelphia, Pa.

Application January 20, 1933. Serial No. 652,587

6 Claims. (Cl. 139—403)

This invention relates to loop pile fabric, and has for an object to provide an improved type of loop forming the pile, wherein the separate threads making up the yarn from which the loops are made react differently to the application of moisture, as for instance, in dyeing.

A further object of the invention is to provide a loop pile fabric, the yarn of which is made up of threads of different properties which react differently to the application of moisture, whereby the finished product discloses upon the surface only one of the threads of the yarn, the other thread being positioned below the surface defined by the first mentioned thread.

15 A further object of the invention is to provide a yarn made up of animal and vegetable threads intertwined, which will react differently to the application of moisture, then weaving the intertwined yarn into a pile fabric in the usual well-known manner, and then dyeing in the piece whereby the animal and vegetable fibre threads are subjected to moisture and to react thereto in accordance with their nature, which differs one from the other.

20 The invention, therefore, comprises the weaving of a loop pile fabric from a yarn made up of one thread of animal fibre and one thread of vegetable fibre, and dyeing the fabric after weaving, the vegetable fibre thread sinking downwardly relative to the loop, while the animal fibre thread extends upwardly relative to the vegetable fibre and in most cases twists upon itself.

In the drawing:—

25 Figure 1 is a view in elevation of a yarn twisted from animal and vegetable fibre threads.

Figure 2 is a diagrammatic view showing the position of the threads after weaving in the usual manner for all pile fabrics, and

30 Figure 3 is a diagrammatic view showing the vegetable fibre thread depressed and widened, and the animal fibre thread upstanding and twisted upon itself.

Like characters of reference indicate corresponding parts throughout the several views.

5 In providing the yarn from which the pile fabric of the present invention is woven, animal and vegetable fibre threads are twisted loosely together. The animal thread may, by way of illustration, be mohair and the vegetable fibre thread likewise referred to as cotton, without in any way limiting the invention to such combination or to either of the components.

At Figure 1 the thread 10 is intended to represent the animal fibre thread while the thread 11 represents the vegetable fibre thread.

At Figure 2 is shown diagrammatically the weave wherein the vegetable fibre thread 11 and the animal fibre thread 10 are formed into the loops 12. This is done upon any type of loom ordinarily employed for weaving loop pile fabric and the invention is in no way limited to the manner of weaving.

There is also diagrammatically shown the threads 13 which represent the foundation. Of course, all of these threads are warp threads and the weft threads are indicated conventionally at 14.

After the fabric is woven to produce the loop pile in the usual manner, the piece is dyed in its entirety. The application of moisture to the animal and vegetable fibre produces a different action of such fibre. For instance, the vegetable fibre 11 mats down and the loops are, consequently, lower than the animal fibre threads 10 which have a tendency to stand up and to twist upon themselves, all of which is shown at Figure 3.

When the animal and vegetable fibres have been subjected to a bath which affects both similarly, it is obvious that they will appear in substantially the same color. However, they may be subjected to baths which affect only an animal fibre or a vegetable fibre, or to two baths of different colors, in which case the vegetable fibre which has matted down forms a background for the animal threads which stand up in pointed relation. This produces an effect quite different from anything heretofore accomplished by reason of the fact that the foundation is scarcely visible, but is obscured by the matted down vegetable threads.

Of course the loop pile fabric herein illustrated may be modified and changed in various ways without departing from the invention herein set forth and hereinafter claimed.

I claim:—

1. A loop pile fabric having loops formed of a yarn composed of both vegetable and animal fibre threads, the vegetable fibre threads in each of said loops being matted down and the animal fibre threads therein standing more erect.

2. A loop pile fabric, each loop of which is constructed of yarn composed of threads of different material, one of which has a tendency to mat down and the other to stand up and twist, following the application of moisture thereto.

3. A loop pile fabric, each loop of which is composed of yarn made up of animal and vegetable threads, reacting differently to the application of moisture.

60

65

70

75

80

85

90

95

100

105

110

4. A loop pile fabric, each loop of which is composed of yarn made up of animal and vegetable fibre threads, the animal fibre threads projecting beyond the vegetable fibre threads.
5. A loop pile fabric, each loop of which is composed of yarn made up of animal and vegetable fibre threads, the vegetable fibre threads being matted down, and the animal fibre threads standing more erect and twisted upon themselves.
- 10
6. The method of producing a loop pile fabric consisting in forming a yarn of threads of animal and vegetable fibre respectively, weaving a loop pile fabric of said yarn, and dyeing the fabric whereby the vegetable fibre threads mat down and the animal fibre threads stand erect and twist.
- 80

FERDINAND W. MOSTERTZ.

85

20

90

25

100

30

105

35

110

40

115

45

120

50

125

55

130

60

140

65

70

75